# EUROPEAN PATENT APPLICATION

(11) **EP 0 234 738 A1**
(43) Date of publication of application: **02.09.1987**
(21) Application number: 87300675.3
(22) Date of filing: 27.01.1987
(51) Int. Cl.: C25D 5/34, C25D 7/10

(54) **Nickel immersion solution and process for electroplating of a bimetal bearing utilizing the same**

(30) Priority: 27.01.1986 IL 77709
(71) Applicant: TECHNO INSTRUMENTS INVESTMENTS 1983 LTD., Bat-Yam 59592 (IL)
(72) Inventor: Relis, Joseph, Ramat Gan (IL); Holtzman, Abraham Moshe, Rehovot (IL)
(74) Representative: Bizley, Richard Edward

(57) **Abstract**

The invention provides an immersion solution for the pretreatment of a bimetal bearing, having one portion thereof composed of an aluminum base metal and another portion of the surface thereof composed of a ferrous base metal, comprising nickel and halogen ions, the solution having an acidic pH. The invention also provides a process for the electroplating of a bimetal bearing having one portion thereof composed of an aluminum base metal and another portion of the surface thereof composed of a ferrous base metal, comprising the pretreatment step of immersing the bearing, prior to the electroplating thereof, in a solution having an acidic pH and containing nickel and halogen ions, whereby the bearing is provided with a coating from the solution without the use of an external source of electricity, which coating can then be coated with an electroplated deposit without any further intermediary steps.

## Description

The present invention relates to the electroplating of bimetal bearings containing aluminum alloys. More particularly, the present invention relates to an immersion bath solution for pretreatment of a composite bearing structure which has one surface composed of an aluminum base metal (i.e., aluminum or an alloy of aluminum) and another surface composed of a ferrous base metal) (i.e., iron or an alloy of iron) prior to the electroplating thereof and to an improved process for electroplating utilizing said immersion hath solution.

As described in U.S. Patent 4.170,525 the deposition of a thin coating or plating on the surface of bearings composed of aluminum or aluminum alloys in order to impart a pleasing appearance thereto or to provide corrosion protection therefor, or to provide a "run-in" surface thereon is well known in the art.

Specifically, it is common practice to apply a thin coating to the surface of a bearing by means of electrodeposition to achieve such results. While this technique has met with success, there are certain inherent disadvantages associated therewith. For example, an electrical power source must be provided and the parts must be properly oriented in the plating bath in order Lo obtain a satasfactory deposit thereon. In addition, an electrodeposition technique also suffers from the fact that it is difficult to apply thin layers of metal to a structure having a complicated surface configuration. Acccordingly, while this technique finds use as a means of applying a thin layer to the surface of a bearing structure it suffers from certain inherent limitations.

Another well known technique for coating the surface of a bearing is the so-called immersion plating process. In this process, metal is deposited from its salt on the surface of the bearing without the aid of an outside source of electrical current or of chemical reducing agents. This process is especially appealing in that thin coatings of uniform thickness can be readily appied to a structure having a complicated surface configuration. Immersion plating baths are either alkaline or acidic. While both types of baths can be used to deposit on the surface of aluminum or aluminum alluy, none of the heretofore known baths can be used to satisfactorily apply a thin coating to a composite structure having one surface composed of an aluminum base metal and another surface composed of a ferrous base metal. Specifically, alkaline immersion baths do not coat both the aluminum and ferrous base metals, but only the aluminum base metal.

Today the most popular commercial system employed in the electro- plating of aluminum and its alloys and bi-metal bearings of iron/ aluminum alloys involves the immersion of parts in an alkaline solution containing Zinc, known as ZINCATE. This process for bearings is described as involving the following steps:
(1) alkaline clean 1
(2) alkaline clean 2
(3) Activation 1
(4) Activation 2
(5) Pickling
(6) Chemical dip in Zincate solution, containing zinc and nickel salts
(7) Immersion in c. 50% Nitric acid solution
(8) Immersion in same Zincate solution as in (6), but with current applied
(9) Activate and neutralize in mild acidic solution
(10) Electrolytic nickel or copper plate to produce a deposit of about 1 micron
(11) Electrolytic lead-tin plate in fluoborate solution to achieve required thickness.

It is to be noted that with rinses after each of the above process steps the complete cycle above contains about twenty-two baths.

It has now been found that contrary to the teaching of the prior art, it is possible to avoid such a tedious and expensive time and chemical consuming multistage process and to obtain bearings having an adherent and uniform electroplated coating by using the novel process and immersion solution of the present invention.

Thus. according to the present invention, there is now provided a process for the electroplating of a bimetal bearing having one portion thereof composed of an aluminum base metal and another portion of the surface thereof composed of a ferrous base metal, comprising the pre- treatment step of immersing said bearing, prior to the electroplating thereof, in a solution having an acidic pH and containing nickel and halogen ions, whereby said bearing is provided with a coating from said solution without the use of an external source of electricity, which coating can then be coated with an electroplated deposit without any further intermediary steps.

In the process of the present invention said electroplated deposit is obtained from the lead fluoborate/tin fiuoborate/copper fluoborate baths typically used in the bearing industry and which are collectively known as 'Babit' solutions.

Alternatively, said electroplated deposit is obtained from lead. lead-tin, tin-lead, nickel, copper, brass, silver, tin, zinc, cadmium. or chromium plating solutions typically used in the metal finishing industry.

U.S. Patent 3,612,964 discloses a process for plating aluminum with an adherent nickel coating by contact with an aqueous solution of hydrofluoric acid and a soluble metal salt such as nickel salt;

U.S. Patent 2,746,136 discloses treatment of aluminum and its alloys prior to electro-plating, wherein aluminum or aluminum base alloys are initially treated by pickling and subsequently coated with a nickel layer by treating in a solution containing a nickel salt and finally electroplated with lead coating;

U.S. Patent 2.580.773 discloses immersing cleaned aluminum or aluminum alloy articles in an aqueous bath containing a water soluble zinc salt and a water soluble fluoride. The electroless metal coating provides a base for receiving a subsequently deposited electrolytic metal layer;

U.S. Patent 2,694,017 discloses nickel plating of aluminum or aluminum alloy materials by immersion in an acetic solution including nickel ions, fluoride ions, phosphite ions and nitrate ions; and

U.S. Patent 3.726.771 discloses a process for chemical nickel plating of aluminum and aluminum alloys wherein the base is electrolessly plated with nickel without extensive pretreatments wherein the nickel is characterized by good adhesion to the aluminum base and which is sufficiently active to allow for direct electrolytic plating without extensive chemical treatments to activate the nickel. The electroless plating solution has an acetic pH and includes nickel ions and fluoride ions.

It is to be noted, however, that none of said patents teaches the nickel coating of an aluminum/iron or aluminum alloy/iron composite bimetal bearing utilizing an immersion bath solution containing Ni⁺² ions and free of reducing agents.

In U.S. Patent 4.170.525 there is described and claimed a method of concurrently coating the surface of a composite bearing structure having one portion of the surface area thereof composed of an aluminum base metal and another portion of the surfce area thereof composed of a ferrous base metal with an adherent layer of tin base metal. comprising:
contacting said composite structure with a mineral acid containing ions selected from the group consisting of fluoride ions, fluoride containing ions or mixtures thereof to activate the surface of said aluminum base metal: and
immersing said composite structure in an aqueous plating bath containing a mineral acid, a source of ions selected from the group consisting of fluoride ions, fluoride containing ions or mixtures thereof and a source of stannous ions with said stannous ions being present in an amount ranging from about 1 to about 75 grams per liter. for a period of time sufficient to cause tin to be deposited concurrently on said aluminum base metal surface by the exchange of aluminum ions for ₜin ions and on said ferrous base metal surface by means of a galvanic couple formed between said aluminum base metal and said ferrous base metal.

Said patent, however, is limited to the use of an immersion solution containing stannous ions which are also considered to be reducing agents and does not teach or suggest a method or solution for coating bimetal bearings with nickel. Furthermore, when example 1 of said patent was repeated using nickel ions instead of stannous ions, no nickel coating was-obtained.

Thus, said patent also does not teach or suggest the immersion solution and method of the present invention.

In a preferred expanded process of the present invention said bearing is subjected to alkaline cleaning and etching followed by neutralization and desmutting prior to immersion in said solution as described hereinafter.

The present invention also provides an immersion solution for the pretreatment of a bimetal bearing having one portion thereof composed of an aluminum base metal and another portion of the surface thereof composed of a ferrous base metal, comprising the pretreatment step of immersing said bearing, prior to the electroplating thereof, comprising nickel and halogen ions, said solution having an acidic pH.

Said solution preferably comprises an acid, such as HC1 or H₂SO₄, to bring the pH of the solution within a range of about 6 to about -0.2 and a solution having a pH range of about 3 to about 0 is especially preferred.

As indicated said solution contains halogen ions, such as F⁻, Cl⁻, BR⁻, I⁻, either individually or in combination, and in individual concentrations up to 160 g/L. and solutions containing chloride or fluorideions and especially solutions containing both fluoride and chloride are preferred.

Said halogen ions are obtained in the solution from readily soluble salts such as NaCl, KCl, LiCl, RbCC1, NH₄C1, KF, KHF₂, NH₄HF₂, HF, NaF and especially preferred are solutions, wherein said halogen ions are derived from an ammonium salt thereof.

Another preferred source of halogen atoms and or the acidic nature of the solution can be the nickel salt which serves as the source of the nickel ions in the solution and thus a solution comprising about 10 to 800 g/1 especially 150 to about 600 g/1 NiCl₂.6H₂O, NiSO₄6H₂O or a combination thereof, is preferred.

Alternatively the solution can·contain between about 0.2 g/1 and 180 g/1 of nickel ions that are provided from nickel salts other than those mentioned above and produced by dissolving nickel metal in an acid or other solution.

An additional preferred component of the solutions of the present invention is an aluminum oxidizing material. Said oxidising materials are typically from the following groups: F⁺⁺⁺, MnO₄, IO₃⁻, IO₄⁻, NO₃⁻, ClO⁻, etc. They can be in the form of simple ions, such as FeCl₃, or complex ions, such as K₃ Fe(CN)₆, especially preferred is an aluminum oxidizing material selected from the group consisting of ferric and permanganate salts.

It is believed that said oxidizing material acts as a promoter to achieve an effective replacement of the aluminum alloy with nickel, thus providing an adherent conversion coating, that is primarily nickel-based and on which an effective and adherent lead-tin coating can be deposited to the required thickness.

As indicated the preferred expanded process of the present invention involves the following process sequence for electroplating of a bi-metal bearing:
(1) cleaning and activating in an alkaline solution;
(2) Neutralisation and desmutting in an acid solution, typically containing nitric acid;
(3) Immersion in the claimed solution without external current.
(4) Electroplating with an electrolytic lead-tin plate fluoborate solution to achieve the required thickness.

Thus the innovative method of coating bi-metal bearing materials of iron/aluminum alloys and aluminum and its alloys prior to further or nickel electrolytic plating in lead-tin / solutions also includes the pretereatment steps of cleaning and etching the parts, which produces a smut on the aluminum alloy surface. This smut is then removed in the acid solution, which typically contains nitric acid, with or without additives depending on the aluminum alloy being employed.

The alkaline solution used for cleaning and etching includes up to 150 g/L of NaOH and up to 200 g/L of proprietary additives and complexors from the groups of EDTA, NTA, DTPA. AGPTA. ethylene diamines, methylene diamines and their derivatives, and also organic acids or their derivatives such as citric acid, tartaric acid, amino acids, gluconic acids, oxalic acids, mallic acids, etc. and salts of acids that are the products of oxidation of carbohydrides, especially the oxidation of the end groups of carbohydrides, such as the aldehyde group and the alcohol group. These organic acid salts are contained in concentrations up to 250 g/L and preferably in concentrations up to 100 g/l. The cleaning and etching solution also contains a wetting agent or surfactant, which is typically non-ionic or anionic and in concentration up to 5%, with a preferred range up to 1.5%.

The neutralisation and desmutting solution typically contains nitric acid in concentrations of between 5% and 100%, with a preferred range of 50% to 100%, the lower range being only limited by the time required to remove the resultant smut from the alkaline cleaning and etching solution. This process is designed to leave the aluminum surface clean and active prior to processing in the innovating immersion solution of the present inventions. If the aluminum alloy contains silicon, it is preferable to also add to the acid neutralisation and desmutting solution salts of the halogen groups, such as F⁻, Cl-, Br⁻, I⁻, either individually or in combination, and in individual concentrations up to 160 g/L, preferably 2 to 60 g/l.

It will be noted that the improved process of the present invention even with rinses after each process step requires only eight baths.

Advantages of the process of the present invention could be summarized as follows:-
(1) As already mentioned above, a much shorter process cycle is required.
(2) There does not exist a normal electrolytic plating requirement in the pre-treatment stages prior to final electrolytic lead-tin plate.
(3) As the immersion solution is acid-based, there is no requirement for a neutralisation step prior to the electrolytic lead-tin plating solution, which is also acid-based.
(4) Excellent adhesion properties of the lead-tin deposit on the aluminum alloy is achieved.
(5) An adherent and uniform deposit thickness up to 50 microns and more is achievable.

The solution also preferably can contain all the metal salts of the metals contained in the bimetals being processed, such as iron salt, aluminum salt, nickel salt, tin salt, copper salt, etc. The purpose of this was found from experiments which clearly showed the solution, which did not initially contain these metal salts, performed better after ageing due to the replacement process.

Thus said solution preferably contains bivalent iron salts, bivalent ion salts and combinations thereof such as FeCl₂, Fe₂(SO₄)₃, PeSO., FeCl₃ etc, preferably in amounts of up to about 150 g/1 iron ions.

The solution preferably also contains a non-ionic wetting agent or surfactant.

While the invention will now be described in connection with certain preferred embodiments in the following examples so that aspects thereof may be more fully understood and appreciated, it is not intended to limit the invention to these particular embodiments. On the contrary, it is intended to cover all alternatives, modifications and equivalents as may be included within the scope of the invention as defined by the appended claims. Thus, the following examples which include preferred embodiments will serve to illustrate the practice of this invention, it being understood that the particulars shown are by way of example and for purposes of illustrative discussion of preferred embodiments of the present invention only and are presented in the cause of providing what is believed to be the most useful and readily understood description of formulation procedures as well as of the principles and conceptual aspects of the invention.

The following examples set forth solutions prepared and tested according to the present invention.

While the solution of Example 1 gave acceptable results, uniformity of coating and grain structure improved with the addition of ingredients in each subsequent example with the solution of example 2 being preferred over the solution of example 1 etc. and the solution of example 6 being most preferred.

### EXAMPLE 1

### EXAMPLE 2

### EXAMPLE 3

### EXAMPLE 4

### EXAMPLE 5

### EXAMPLE 6

While the composition of example 6 represents an especially preferred and commercial immersion solution according to the present invention further components can be added thereto to meet customer specifications and to further improve the properties thereof.

Thus said solution can also preferably contain metallic brighteners from the group, such Zn, Cd, Pb, and Thalium in the form of one of their salts of complexes, and in concentration up to 5 grams of metal per liter.

The solution can also preferably contain organic brighteners which can also be included to provide stress-relieving, said brighteners including imide derivatives such as ortho-benzoic sulphonimide, benzene sulphonimide, bi-dibenzene sulfonimide, heterocyclic sulphonic acids such as thiophen-2- sulphonic acid, aromatic sulphinic acids such as benzene sulphinic acid, ethylenic aliphatic sulphonic acids such as allyl sulphonic acid. aromatic sulphonic acids such as benzene suphonic acid, aromatic sulphonamides such as paratoluene sulphonamide.in concentrations up to 10 g/L.

The following further solutions according to the present invention were also prepared each solution incorporating several of the following 20 possible components, set forth hereinafter in amounts of g/l.

Of the following compositions, that of Example 13, is especially preferred.

The following example describes an electroplating process according to the present invention.

### EXAMPLE 14

An aluminum alloy bearing conforming to SAE standard J460e and containing 78.3% aluminum and 20% tin is first placed in an alkaline bath for 1 to 3 minutes at a temperature of between 25 to 50°C for cleaning and surface activation. The bearing is then removed and washed with water.

After rinsing the bearing is placed in a nitric acid bath for 20 to 90 seconds at room temperature (20 - 30°C). The nitric acid bath desmutes the surface of the bearing and leaves it clean and active.

The bearing is then once again rinsed in a water bath for 1-2 minutes.

The rinsed bearing is then placed in a solution according to the present invention for 1 to 3 minutes at room temperature.

The bearing is then rinsed again in water and placed in an electroplating bath containing lead fluoborate. tin fluoborate, copper fluoborate and fluoboric acid having a preferred ratio of 90% lead fluoborate : 92 tin fluoborate : 1 % copper fluoborate.

The current density of the electroplating bath is up to about 6 amper/dm² and the voltage is about 0.4-6 volts. The electroplating is carried out at 20 - 60 °C for up to 30 minutes using a lead tin anode (90% Pb : 10% Sn) using direct or preferably pulsed current.

The resulting bearing has a uniform plating of about 12-50 microns.

After the pretreatment step of the present invention. the bearing can alternatively be plated with nickel from a Wattes Nickel bath containing 300-330 g/1 nickel sulphate. 60-80 g/1 nickel chloride and 35-45 g/1 Boric acid, or other nickel bathes.

In this nickel plating process the current density used is up to 10 ampers/dm², the voltage is about 6-8 volts, the temperature is preferably about 40⁰⁻60⁰C and the anode is made of nickel.

It will be evident to those skilled in the art that the invention is not limited to the details of the foregoing illustrative examples and that the present invention may be embodied in other specific forms without departing from the essential attributes thereof, and it is therefore desired that the present embodiments and examples be considered in all respects as illustrative and not restrictive. reference being made to the appended claims, rather than to the foregoing description, and all changes which come within the meaning and range of equivalency of the claims are therefore intended to be embraced therein.

## Claims

1. An immersion solution for the pretreatment of a bimetal bearing, having one portion thereof composed of an aluminum base metal and another portion of the surface thereof composed of a ferrous base metal, comprising nickel and halogen ions, said solution having an acidic pH.

2. An immersion solution according to claim 1, further comprising an acid to bring the pH of the solution within a range of about 6 to about -0.2.

3. An immersion solution according to claim 1, having a pH of about 3 to about 0.

4. An immersion solution according to any one of claims 1 to 3, wherein said halogen ions are chloride ions or fluoride ions or a combination of chloride and fluoride ions.

S. An immersion solution according to any one of claims 1 to 4, wherein said halogen ions are derived from an ammonium salt thereof or from a potassium or sodium salt thereof.

6. An immersion solution according to any one of claims 1 to 5, further comprising an aluminum oxidizing material, e.g. a ferric and/or permanganate salt.

7. An immersion solution according to any one of claims 1 to 6, further comprising bivalent iron salts, trivalent iron salts and combinations thereof, and/or copper ions.

8. An immersion solution according to claim 7, comprising up to about 150 g/1 of said iron ions.

9. An immersion solution according to any one of claims 1 to 8, comprising about 10 to about 800 g/1 NiCl₂.6H₂O, NiSO₄6H₂O or a combination thereof.

10. An immersion solution according to any one of claims 1 to 9, comprising up to about 260 g/1 halogen ions.

11. An immersion solution according to any one of claims 1 to 10, further comprising up to about 30 g/1 of a wetting agent or surfactant.

12. An immersion solution according to any one of claims 1 to 11, further comprising metallic brighteners selected from the salts and complexes of zinc, cadmium, lead and thallium.

13. An immersion solution according to any one of claims 1 to 12, further comprising soluble metal salts corresponding to the metal components of said bimetal bearing.

14. A process for the electroplating of a bimetal bearing having one portion thereof composed of an aluminum base metal and another portion of the surface thereof composed of a ferrous base metal, comprising the pretreatment step of immersing said bearing, prior to the electroplating thereof, in a solution having an acidic pH and containing nickel and halogen ions, whereby said bearing is provided with a coating from said solution without the use of an external source of electricity, which coating can then be coated with an electroplated deposit without any further intermediary steps.

15. A process according to claim 14, wherein said electroplated deposit is provided by a lead fluoborate, tin fluoborate or copper fluoborate solution.

16'. A process according to claim 14, wherein said electroplated deposit is provided by a lead, lead-tin, tin-lead, nickel, copper, brass silver, tin, zinc, cadmium or chromium plating solution.

17. A process according to any one of claims 14 to 16, wherein said bearing is subjected to alkaline cleaning and etching following by neutralization and desmutting prior to immersion in said solution.
